

## UNITED STATES PATENT OFFICE

WACLAW IWANOWSKI AND JOZEF TURSKI, OF WARSAW, POLAND

## IMPREGNATION OF WOOD AND OTHER VEGETABLE SUBSTANCES

No Drawing. Application filed June 6, 1927, Serial No. 196,998, and in Poland August 13, 1926.

Phenol, its homologues and different derivatives have been known for some time as antiseptics and are used for wood preserving. The present invention consists essentially in 5 the use for wood impregnating purposes, of poly-chlor derivatives of phenol and their homologues, that is to say of the di-, tri- and other poly-chlorinated derivatives with the chlorine in the benzene nucleus. These poly-chlor derivatives are greatly superior in 10 regard to their activity against wood-destroying fungi, to the non-chlorinated and mono-chlorinated phenols.

In addition, di-chlor derivatives do not increase the inflammability of the wood impregnated therewith and the tri- and other poly-chlorinated derivatives counteract this inflammability to a very great extent.

For wood impregnating purposes, use 20 should be made preferably of aqueous solutions of the poly-chlor phenols or their salts, alone or mixed with other impregnating agents. It is sufficient to impregnate with a 0.07-0.1% solution.

25 Nitro-chlor-phenols and the condensation products of chlor-phenols with arsenic chloride are equally well suited for this purpose.

In the appended claims, unless otherwise indicated, the word "phenol" designates the 30 compound  $C_6H_5OH$  and its homologues, "phenol compound" designates the free phenol and its homologues and their salts, and "poly-chlorinated" designates compounds containing more than one chlorine 35 atom to the molecule, the word "chlorinated" being generic to mono- and poly-chlorinated compounds.

Having now more particularly described 40 and ascertained the nature of our said invention and in what manner the same is to be performed we declare that what we claim is:

1. Process of preserving wood which comprises impregnating the wood with a chlorinated phenol compound containing at least 45 two and not more than three chlorine atoms.

2. Process of preserving wood which comprises impregnating the wood with a chlorinated nitro-phenol compound.

3. Process of preserving wood which comprises impregnating the wood with a chlorinated phenol condensed with an arsenic chloride. 50

Dated this 28th day of April 1927.

WACLAW IWANOWSKI.  
JOZEF TURSKI.

55

60

65

70

75

80

85

90